# EUROPEAN PATENT APPLICATION

(11) **EP 0 994 214 A1**
(43) Date of publication of application: **19.04.2000**
(21) Application number: 98203426.6
(22) Date of filing: 12.10.1998
(51) Int. Cl.: D06P 1/00

(54) **Process for printing on cloth with watersensitive colors**

(71) Applicant: Taroko Textile Corporation, Taipei (TW)
(72) Inventor: Hsieh, Rea-Cheng, Taipei (TW)
(74) Representative: Smulders, Theodorus A.H.J., Ir.

(57) **Abstract**

The present invention relates to a process for producing an aqua printing on cloth which makes the designs and/or patterns appear thereon when coming in contact with water. In the present invention, special materials are mixed to form an aqua printing paste with their fixed percentages. The aqua printing paste is coated on the surface of the cloth according to the designs on a screen and then is dried to form a film. At high temperature, a crosslinking bond is formed between the materials and fiber of the cloth. After the uncrosslinking materials are washed off, the designs and/or patterns will become visible when they come in contact with water.

## Description

The present invention relates to a process for producing aqua printing on cloth. More particularly, the present invention relates to a process for producing aqua printing on cloth where the figures and/or patterns will appear when they come in contact with water.

The process for producing aqua printing on cloth according to the present invention basically comprises the steps of:
- Preparing an aqua printing paste;
- Printing the aqua printing paste in a design and/or pattern onto a selected area of the surface of the cloth using a silk screen technique; then
- Curing and fixing the aqua printing paste applied to the surface of the cloth to form a film; and
- Washing.

During curing and fixing, crosslinking bonds are formed between the selected components contained in the aqua printing paste and the fiber of the cloth. The components not bonded with the fiber of the cloth are washed off with water. Then the design and/or pattern on the selected area of the cloth surface will be visible when they are wet with water.

The present invention also relates to a process of producing aqua printing a white pattern on cloth, which comprises the steps of:
- Preparing an aqua printing paste;
- Preparing a white pigment paste;
- Subsequently printing the aqua printing paste and the white pigment paste designs and/or patterns onto selected areas of the surface of the cloth using silk screen techniques; then
- Curing and fixing the aqua printing paste and the white pigment paste applied to the surface of the cloth to form films; and
- Washing.

Furthermore, the aqua printing on cloth according to the present invention can be treated with a water-proof process by coating the surface of the cloth with a liquefied polyurethane resin (PU) or acrylic resin so that a film is formed thereon, resulting in a water-proof and air-tight effect.

The aqua printing on cloth of the present invention is typically used near or in water. Consequently, it is used in the manufacture of items such as tablecloths, swimming suits, beachwear, umbrellas, handkerchiefs, towels, tents, jackets, and tarpaulins.

The aqua printing on cloth of the present invention can be used to display different designs in wet or dry situation. Thus, the collocation of the color and design of the aqua printing on cloth according to the present invention may produce an unconventional effect. The aqua printing on cloth of the present invention also can show whether an item is dry or not. This is not only helpful in distinguishing its state but also in deciding whether it needs be further dried.

It is an object of the present invention to provide a process for producing aqua printing on cloth.

It is another object of the present invention to provide a process for producing aqua printing on cloth, such that the designs will appear when they are wet.

It is yet another object of the present invention to provide a process of producing aqua printing on cloth with white designs and/or patterns.

It is another object of the present invention to provide a process of manufacturing aqua printing on cloth with waterproof and insulating qualities.

The process for producing aqua printing on cloth of the present invention comprises the steps of:
- Preparing an aqua printing paste;
- Printing the aqua printing paste in a design and/or pattern onto a selected area of the surface of the cloth by a silk screen technique ; then
- Curing and fixing the aqua printing paste on the surface of the cloth to form a film; and
- Washing.

If necessary, the aqua printing on cloth according to the present invention can be treated with a waterproof process, so as to make the aqua printing on cloth waterproof. Basically, the waterproof process comprises the steps of coating glue on one or both surfaces of the cloth and curing the glue.

The present invention also relates to a process of aqua printing a white pattern on cloth, which comprises the steps of:
- Preparing an aqua printing paste;
- Preparing a white pigment paste;
- Subsequently printing the aqua printing paste and the white pigment paste designs and/or patterns onto selected areas of the surface of the cloth by silk screen techniques; then
- Curing and fixing the aqua printing paste and the white pigment paste on the surface of the cloth to form films; and
- Washing.

The present invention is further specified by the following preferred embodiments. Unless indicated otherwise, the following percents are calculated based on weight.

### Preparation of Aqua Printing Paste

The aqua printing paste is composed of:

| | |
|---|---|
| a. Aqua printing source paste | 95% |
| 1. emulsifier, | 5% |
| 2. water, | 45%, |
| 3. high-flash aromatic naphtha, | 50% |
| b. Water repellant | 5% |

Water repellants are a well-known product in this art and most of them are commercially available, such as FC-270 supplied by PROPULSION CO. Ltd., Taiwan.

The aqua printing paste is manufactured by uniformly mixing 95% aqua printing source paste and 5% water repellent (FC-270), wherein the aqua printing source paste is formed by mixing and emulsifying 5% emulsifier, 45% water and 50% high-flash aromatic naphtha at a mixer velocity of 1500-2000 rpm.

### Preparation of White pigment Paste

### Preparation of the Source Paste

The white pigment paste is composed of:

| | |
|---|---|
| a. Source paste | 40% |
| 1. fixing agent, (ACRAMIN PUD, supplied by BAYER, Taiwan) | 40% |
| 2. sodium hexametahposphate, | 0.1% |
| 3. emulsifier VA, | 1.17% |
| 4. emulsifier WV, (Supplied by CHIN YEE CHEMICAL INDUSTRIES LTD., Taiwan) | 1.5% |
| 5. diethylene glycol, | 8% |
| 6. crosslinking agent, (ACRAFIX MF supplied by BAYER, Taiwan) | 5% |
| 7. high-flash aromatic naphtha, (Miao No. 1, supplied by CHINESE PETROLEUM CORPORATION., Taiwan) | 5% |
| 8. water, | 37.33% |
| 9. synthetic paste, ( ACRACONZ BN, supplied by BAYER, Taiwan) | 1.9% |
| b. white pigment, (Pigment DRN) | 60% |

0.1% sodium hexametahposphate, 1.17% emulsifier VA and 1.5% emulsifier WV are mixed with 8% diethylene glycol, 6% crosslinking agent (ACRAFIX MF), 37.33% water and 1.9% synthetic paste (ACRACONZ BN), then is uniformly stirred to form a uniform mixture. 5% high-flash aromatic naphtha (Miao No. 1) is slowly added into the mixture while stirring is continued at a velocity of 1500-2000 rpm. After the mixture is completely emulsified, the fixing agent (ACRAMIN PUD) is added to form a source paste.

The white pigment paste is manufactured by mixing 40% source paste and 60% white pigment (Pigment DRN).

### Printing

There are two printing processes. One is flat-screen printing, the other is rotary-screen printing. The screens used for the aqua printing paste and white pigment paste are different. The screen suitable for the aqua printing paste is 1800 mesh; and the screen suitable for the white pigment paste is 1000 mesh.
a. If the flat-screen process is used, the following requirements are applied:
   Speed of the cloth: 13 meter/min;
   Temperature of drying: 130°C;
   Length of the scraper: 2.8 cm;
b. If a rotary-screen process is used, the following requirements are applied:
   Speed of the cloth: 45 meter/min;
   Temperature of drying: 130°C;
   Angle between the scraper and the cloth: +5° ;

### Curing and Fixing

After printing, the cloth is cured and fixed at a condition of 180°C x 60 meter/min (overfeed stuff +3%). During curing and fixing, the materials printed on the cloth react with the fiber of the cloth to form crosslinking bonds.

### Washing

After drying, the cloth is washed with water at a speed of 30 meter/min (80°C) without adding any additives to remove all the unreacted materials.

### Drying

After washing, the cloth can be optionally dried. Preferably, the temperature for drying is 120°C.

The materials used in the present process are described as follows:

The fixing agent (ACRAMIN PUD) is an anion dispersion of polyurethane polyester of fatty series. This fixing agent is suitable for the situation where the source paste either contains very little high-flash aromatic naphtha or doesn't contain any high-flash aromatic naphtha. Additionally, this fixing agent makes textiles flexible.

The emulsifier (Emulsifier VA) is a non-ionic derivative of polyethylene glycol, which promotes the uniformity of the printed color, reduces the sensibility of kneading, increases the osmosis ability of the paste and promotes the fluidity of the paste. It also has a preferable resistance to electrolytes, acids and bases.

The emulsifier (Emulsifier WA) is a non-ionic derivative of aryl polyethyldiether, which increases the fluidity of the paste during printing color and can be easily removed during the period of washing the screen. It also has a preferable resistance to electrolytes, acid, base and hardwater.

Diethylene glycol increases the smoothness of the color printing paste, decreases clogging the screen and promotes the softness of the paste film formed on the cloth.

The crosslinking agent (ACRAFIX MF) is a colorless liquid of etherfied melamine resin, which forms a multi-functional crosslinking bond and promotes the adhesive effect of the film during washing. Additionally, it has preferable fluidity.

The high-flash aromatic naphtha is an oil produced by MiaoLi Oil Plant of China, named Miao No. 1, which is the emulsified oil in oil and water solution.

The synthetic paste (ACRACONQ BN) is a copolymer of ammonium salt of the acrylic series, which have preferable properties of resisting electrolysis and hardwater. Additionally, it promotes the chromaticity value and uniformity of the printing, and is also easily processed and washed off after printing. Furthermore, the designs and/or patterns on the cloth surface look clearer.

Sodium hexametahposphate is a water-processing agent which ensures the quality of water.

The emulsifier (PE MET) helps water and the high-flash aromatic naphtha (Miao 1) to combine with each other by destroying the boundary tension between the water and the high-flash aromatic naphtha.

The water repellent (FC-270) is a positive ions' water repellent of fluorine series, which produces an oil repelling and water-repelling effect.

The techniques associated with making the aqua printed designs and/or patterns according to the present invention appear on the cloth when coming in contact with water could be categorized as follows:
1. The fibers, which have designs and/or patterns printed thereon and treated with water repellent, have a good water-repellant characteristic. When the cloth comes in contact with water, the treated fibers remain dry, and the fibers which are not treated with water repellent adsorb water, thus the designs and/or patterns appear on the surface of the cloth.
2. The fiber of the cloth except for the surface printed with designs and/or pattern is treated with the water repellent. When the fibers printed with designs and/or patterns absorb water and the other fibers still remain dry, the designs and/or patterns appear on the surface of the cloth.

### Waterproof Treatment

Furthermore, the cloth with aqua printing according to the present invention can be treated with a waterproof process so as to make the aqua printing cloth waterproof.
The agents that can be used for the waterproof treatment are:
Polyurethane resin (RS-25CD, supplied by Yu Feng Chemical Industry Co. Ltd., Taiwan) is the main component used in one of the waterproof treatments. It has the properties of preferable extension ratio, stretching resistance and softness.
Acrylic resin (TOA ACRON, supplied by TOA RESIN CORPORATION LIMITED, Taiwan) is the main component used in another one of the waterproof treatments. It has the properties of preferable extension ratio, stretching resistance and softness.
Crosslinking agent (DC-75, supplied by DYNASTY CHEMICAL INDUSTRIES CO. LTD., Taiwan) is used in combination with polyurethane resin, which increases the heat resistance, corrosion resistance and tackiness of the formed film on the cloth.
Crosslinking agent (CL-3, supplied by LIDYE CHEMICAL CO. LTD., Taiwan) is used in combination with acrylic resin, which increases the heat resistance, corrosion resistance and tackiness of the formed film on the cloth.
Surface conditioner (CRISVON ADDITIVE No.5, supplied by LIDYE CHEMICAL CO. LTD., Taiwan) is suitable as a surface additive for cloth.
Butanone( MEK) is a solvent used for diluting polyurethane (PU) resin.
Toluene is a solvent used for diluting acrylic resin.

### Formulation used in the waterproof treatment:

| A. With respect to polyurethane resin | |
|---|---|
| (1) Bottom coating glue: | |
| Polyurethane glue (RS-25CD): | 77% |
| Crosslinking agent (DC-75): | 1% |
| Solvent (M.E.K): | 22% |

| (2) Top coating glue: | |
|---|---|
| a. Polyurethane resin ( RS-25CD): | 54.3% |
| Surface conditioner (CRISVON ADDITIVE No.5): | 1.4% |
| Corsslinking agent (DC-75): | 0.9% |
| Solvent (M.E.K): | 20.8% |
| Color glue*: | 22.6% |
| b. Polyurethane (PU) resin (RS-25CD): | 67% |
| Surface conditioner (CRISVON ADDITIVE No.5): | 1% |
| Crosslinking agent (DC-75): | 1% |
| Solvent (M.E.K): | 25.7% |
| Gold or silver powder: | 5.3% |
| c. Polyurethane resin ( RS-25CD): | 70% |
| Surface conditioner (CRISVON ADDITIVE No.5): | 1% |
| Crosslinking agent (DC-75): | 1 % |
| Solvent (M.E.K): | 28 % |

| A. With respect to the acrylic resin | |
|---|---|
| (1) Bottom coating glue: | |
| 16% acrylic resin: | 98.8% |
| Crosslinking agent (CL-3): | 1.2% |

| (2) Top coating glue: | |
|---|---|
| 16% acrylic resin: | 60% |
| Crosslinking agent (CL-3): | 1% |
| Surface conditioner (CRISVON ADDITIVE No.5): | 1% |
| Solvent (Toluene): | 26% |
| Color glue* or glue containing copper/silver: | 12% |

| | |
|---|---|
| *This color glue is a commercially available coating glue of any color. | |
| *This color glue is commercial available coating glue of being miscible to acrylic resin. | |

### Manufacture of glue:

Preparation of the bottom coating glue:
   After the polyurethane (PU) or acrylic resin is uniformly mixed, the crosslinking agent is added slowly. Then, the mixture is stirred at a stirrer speed of 1500∼2000RPM for 10 minutes.
Preparation of the top coating glue:
   The solvent is firstly mixed with the color glue or the glue containing copper/silver by a stirrer for 5 minutes. Then, the PU or acrylic resin is added and uniformly stirred. Thereafter, the surface conditioner is added and the mixture is uniformly stirred at a speed of 1500∼2000RPM.
Coating:
Coating of the bottom coating glue:
The bottom coating glue is coated at the following conditions:
Speed: 30 meters/min,
Temperature: 160°C.
The top coating glue is coated at the following conditions:
Speed: 30 meters/min,
Temperature: 160°C .

Although the present invention has been described with reference to preferred embodiments, the embodiment is only for the purpose of puffing on a demonstration rather than limiting the invention. Workers skilled in the art will recognize that changes may be made in form and detail without departing from the spirit or essential attributes thereof.

## Claims

1. A process for producing aqua printing on cloth, comprises the steps of:
- Preparing a aqua printing paste;
- Printing the aqua printing paste in design and/or pattern onto a selected area of the surface of the cloth by a silk screen technique; then
- Curing and fixing the aqua printing paste to form a film on the surface of the cloth; and
- Washing.

2. A process for producing a white pattern aqua printing on cloth, comprises the steps of:
- Preparing a aqua printing paste;
- Preparing a white pigment paste;
- Subsequently printing the aqua printing paste and the white pigment paste in designs and/or patterns onto selected areas of the surface of the cloth by silk screen techniques having; then
- Curing and fixing the aqua printing paste and the white pigment paste to form films on the surface of the cloth; and
- Washing.

3. The process of claim 1 or 2, wherein the aqua printing paste is composed of:
| | |
|---|---|
| a. Aqua printing source paste | 95% |
| 1. emulsifier, | 5% |
| 2. water, | 45%, |
| 3. high-flash aromatic naphtha, | 50% |
| b. Water repellant | 5%. |

4. The process of claim 2, wherein the white pigment paste is composed of:
| | |
|---|---|
| a. Source paste | 40% |
| 1. fixing agent, | 40% |
| 2. sodium hexametahposphate, | 0.1% |
| 3. emulsifier VA, | 1.17% |
| 4. emulsifier WV, | 1.5% |
| 5. diethylene glycol, | 8% |
| 6. crosslinking agent, | 5% |
| 7. high-flash aromatic naphtha, | 5% |
| 8. water, | 37.33% |
| 9. synthetic paste, | 1.9% |
| b. white pigment, | 60% |

5. The process of claim 1 or 2, where a waterproof process is optionally applied.

6. The process of claim 5, wherein the waterproof process applies polyurethane-containing formulation or acrylic-containing formulation.

7. The process of claim 6, wherein the polyurethane-containing formulation comprises bottom coating glue and top coating glue.

8. The process of claim 7, wherein the bottom coating glue is composed of:
| | |
|---|---|
| Polyurethane glue: | 77% |
| Crosslinking agent: | 1% |
| Solvent : | 22% |

9. The process of claim 7, wherein the top coating glue is composed of:
| | |
|---|---|
| a. Polyurethane resin: | 54.3% |
| Surface conditioner: | 1.4% |
| Corsslinking agent: | 0.9% |
| Solvent: | 20.8% |
| Color glue: | 22.6% |
| b. Polyurethane resin: | 67% |
| Surface conditioner: | 1% |
| Crosslinking agent: | 1% |
| Solvent: | 25.7% |
| Gold or silver powder: | 5.3% |
| c. Polyurethane resin: | 70% |
| Surface conditioner: | 1% |
| Crosslinking agent: | 1 % |
| Solvent: | 28 % |

10. The process of claim 6, wherein the acrylic-containing formulation comprises bottom coating glue and top coating glue.

11. The process of claim 11, wherein the bottom coating glue is composed of:
| | |
|---|---|
| 16% acrylic resin: | 98.8% |
| Crosslinking agent: | 1.2% |

12. The process of claim 11, wherein the top coating glue is composed of:
| | |
|---|---|
| 16% acrylic resin: | 60% |
| Crosslinking agent: | 1% |
| Surface conditioner: | 1% |
| Solvent: | 26% |
| Color glue or glue containing copper/silver: | 12% |
